

## UNITED STATES PATENT OFFICE

1,995,615

## MOTOR FUEL

Alphons O. Jaeger, Mount Lebanon, Pa., assignor,  
by mesne assignments, to American Cyanamid  
& Chemical Corporation, a corporation of  
Delaware

No Drawing. Application September 1, 1931,  
Serial No. 560,665

3 Claims. (Cl. 44—9)

This invention relates to motor fuels and more particularly to motor fuels containing gum-forming unsaturated compounds such as, for example, cracked gasoline. These fuels are highly desirable because of their excellent anti-knock properties, but the tendency to form a colored gum, especially under the influence of sunlight, renders them objectionable particularly where they are sold in the so-called visible dispensing pumps and are subject to the action of sunlight.

It has been proposed to stabilize the fuel by the addition of components which tend to prevent the formation of the colored gums. In the past, two such stabilizers have been described, namely, anthracene, phenanthrene and phenols and acid amines of aromatic amines such as acetanilide. I have found that esters of carboxylic acids are good stabilizers. While the lower molecular esters such as esters of fatty acids may be used with effect, the esters of higher molecular acids and particularly polybasic acids and keto aromatic acids are preferable.

Among the esters of aliphatic acids are the alkyl esters of formic, acetic, propionic, butyric, etc., particularly esters of the higher alcohols such as the butyl and amyl esters, including the esters from the mixed amyl alcohols obtained by the hydrolysis of chlorinated pentanes from natural gas and sold on the market under the name of "Pentasol". Glycerin esters are less effective than the esters of mono and dihydric alcohols but are included in the invention in its broader aspects.

A very effective class of aliphatic esters are those of the dibasic acids, such as oxalic, maleic, fumaric, malic, succinic, tartaric, citric, adipic, etc.

The esters of aromatic acids are very desirable, particularly the phthalates, benzoates and esters of the keto aromatic acids such as benzoylbenzoate, naphthoylbenzoate, and their substitution products. Esters of amino substituted aromatic acids are particularly effective, for example esters of aminophthalic, anthranilic, para-aminobenzoic, aminonaphthoic, etc.

Esters of hydroxy acids are also useful, such as lactates, salicylates, and the like and the dibasic hydroxy acids such as malic and tartaric referred to above.

Another group of esters are those of the heterocyclic acids such as pyromucic, various pyridine and quinolin carboxylic acids, and the like.

The invention will be described in greater de-

tail in connection with the following specific examples:

*Example 1*

2-6 pounds of "Pentasol" acetate are mixed with 100 barrels of cracked gasoline, producing a well stabilized product. 5

*Example 2*

2½-5 pounds of methyl anthranilate are added to 100 barrels of cracked gasoline, producing a motor fuel of good stability. 10

*Example 3*

2-5½ pounds of dibutyl phthalate are mixed with 100 barrels of cracked gasoline, resulting in a well stabilized motor fuel. 15

*Example 4*

3-6 pounds of ethyl benzoylbenzoate are added to 100 barrels of gasoline, resulting in a product of satisfactory stability. 20

*Example 5*

3-5½ pounds of dimethyl maleate are added to 100 barrels of gasoline. A well stabilized gasoline is obtained. 25

*Example 6*

2-6 pounds of methyl pyromucate are mixed with 100 barrels of gasoline, a thoroughly stabilized product being obtained. 30

*Example 7*

3-5 pounds of benzylbenzoate are added to 100 barrels of gasoline. A product of satisfactory stability is obtained. 35

*Example 8*

A mixture of 2½ to 6 pounds of diethyl phthalate and urea are added to 100 barrels of gasoline, producing a well stabilized product. 40

*Example 9*

A mixture of 3-5½ pounds of butyl naphthoylbenzoate and acetanilide are mixed with 100 barrels of gasoline, resulting in a well stabilized motor fuel. 45

*Example 10*

2-5 pounds of a mixture of ethyl ester of 2-phenyl quinolin 4-carboxylic acid and anthracene are added to 100 barrels of gasoline. A product of satisfactory stability is obtained. 50 55

It will be apparent from the examples that not only can the esters of carboxylic acids be used alone, but they may be used in conjunction with other stabilizers of different types. Naturally, 5 of course, a plurality of esters of carboxylic acids may be used.

While it is normally desirable to use as little stabilizer as possible and the examples show 10 amounts of stabilizer on the order of a few hundredths of a percent, larger amounts of stabilizer may, of course, be used, without any harm, but practically the amount of stabilizer never need exceed 1% and preferably the amount used is from .01% to 1%.

What is claimed as new is:

1. A cracked motor fuel normally tending to deteriorate on storage to which has been added an ester of an unsaturated di-carboxylic acid in quantities sufficient to retard such deterioration. 5

2. A cracked motor fuel normally tending to deteriorate on storage to which has been added a phthalate ester in quantities sufficient to retard such deterioration. 10

3. A cracked motor fuel normally tending to deteriorate on storage to which has been added a maleate ester in quantities sufficient to retard such deterioration.

ALPHONS O. JAEGER.